



US006305458B1

(12) **United States Patent**  
Gligor

(10) **Patent No.:** US 6,305,458 B1  
(45) **Date of Patent:** Oct. 23, 2001

(54) **LOST FOAM AND SAND CORES STAGE  
MANUFACTURING TECHNOLOGY**

(75) Inventor: **Corneliu Ioan Gligor**, Tulsa, OK (US)

(73) Assignee: **Baker Hughes Incorporated**, Houston, TX (US)

(\*) Notice: Subject to any disclaimer, the term of this patent is extended or adjusted under 35 U.S.C. 154(b) by 0 days.

(21) Appl. No.: **09/526,324**

(22) Filed: **Mar. 15, 2000**

**Related U.S. Application Data**

(60) Provisional application No. 60/124,898, filed on Mar. 17, 1999.

(51) **Int. Cl.<sup>7</sup>** ..... **B22C 9/22**

(52) **U.S. Cl.** ..... **164/34; 164/28**

(58) **Field of Search** ..... 164/34, 28, 30, 164/32, 108, 112

(56) **References Cited**

**U.S. PATENT DOCUMENTS**

|            |        |                            |
|------------|--------|----------------------------|
| Re. 31,488 | 1/1984 | Trumbauer .                |
| 3,889,737  | 6/1975 | Olsen .                    |
| 4,078,598  | 3/1978 | Kelso et al. .             |
| 4,243,093  | 1/1981 | Nieman ..... 164/96        |
| 4,285,385  | 8/1981 | Hayashi et al. ..... 164/9 |
| 4,462,453  | 7/1984 | Trumbauer ..... 164/32     |
| 4,691,754  | 9/1987 | Trumbauer et al. .         |

|           |         |                              |
|-----------|---------|------------------------------|
| 4,736,786 | 4/1988  | Trumbauer et al. .           |
| 5,027,878 | 7/1991  | Revankar et al. ..... 164/98 |
| 5,063,992 | 11/1991 | Mrdjenovich et al. .         |
| 5,372,176 | 12/1994 | Brown et al. ..... 164/34    |
| 5,755,271 | 5/1998  | Williamson .                 |

*Primary Examiner*—Tom Dunn

*Assistant Examiner*—Len Tran

(74) *Attorney, Agent, or Firm*—Bracewell & Patterson, LLP.

(57) **ABSTRACT**

A method of casting a workpiece having internal cavities uses a combination of sand core and lost foam techniques. A core of bonded granular material in the desired configuration of the voids of the workpiece is formed. The core has oppositely facing first and second surfaces with a pattern of channels extending between them. The pattern of the channels is in the desired configuration of walls for the cavities of workpiece. A first foam layer of destructible material is preformed and secured to the first surface of the core overlying one side of the channels. A second foam layer of destructible material is preformed and secured to the second surface of the core, overlying an opposite side of the channels. The assembly is placed in a refractory mold cavity, and granular refractory material is packed around the assembly. Molten metal is poured into the mold cavity into contact with the first and second foam layers, which decompose, causing the molten metal to flow into the channels, forming metal walls for the workpiece in the channels and in the spaces previously occupied by the foam layers.

**16 Claims, 3 Drawing Sheets**





Fig. 1



Fig. 2



Fig. 3



Fig. 4



Fig. 5



Fig. 6



Fig. 7

## LOST FOAM AND SAND CORES STAGE MANUFACTURING TECHNOLOGY

### RELATED APPLICATION

Applicant claims priority to provisional application Ser. No. 60/124,898 filed Mar. 17, 1999.

### TECHNICAL FIELD

The present invention relates to a foundry tooling process and method using destructible material in casting operations for producing complex internal shapes requiring a high degree of surface finish. More particularly, the invention relates to a process for producing impellers and diffusers for centrifugal submersible pumps.

### BACKGROUND OF THE INVENTION

Many cast parts require the formation of voids therein. An example of such castings includes impellers of pump stages in centrifugal submersible pumps.

One method for forming such castings is the lost foam method. In the lost foam method, consumable patterns, such as polystyrene foam plastic, are coated with a permeable refractory wash and then embedded in foundry sand to be replaced by molten metal. The molten metal vaporizes the foam-type pattern and a metal duplicate of the pattern is the result. The lost foam method is advantageous because it allows for net shape capacity, i.e., the ability to produce a finished or near-finished casting that requires little or no machining. However, the lost foam method is unsuitable for the geometric particularities of the hydraulic passages required in complex castings, such as impellers and diffusers. The lost foam process is not suitable to form some complex castings because of process shortcomings including limitations in thickness of the walls as well as major costs associated with tooling, low consistency in the molding stage, low surface finish and low compression strength. Additionally, particular types of geometries result in warping of the castings. Therefore, such castings do not achieve a near net shape.

Another method for forming castings is sand molding. Sand molding uses high strength chemically bonded sand. Sand molding is not a preferred choice to form net shape parts because of mold wall movement. Additionally, some specific requirements of sand molding may only be met by high quality foundries.

Therefore, it is desirable to develop a method that results in near net shape, that is low in cost, and that avoids the shortcomings of the lost foam process. One solution is proposed in U.S. Pat. No. 4,691,754, which teaches molding a destructible layer around a first core by placing the first core into a molding machine. Partially pre-expanded polystyrene pellets are applied to the core and fully expanded, via a steam expansion step. However, a drawback with this method is that the core is exposed to moisture during the steam expansion step. It is desirable to avoid exposing the core, which is typically hygroscopic, to moisture. If the core is exposed to moisture, molten metal will come in contact with the moisture absorbed by the core when the molten metal is poured into the core. The exposure of molten metal to moisture is undesirable.

### SUMMARY OF THE INVENTION

A casting method that combines a lost foam method and a sand molding method provides desired benefits without undesirable effects. The present invention is a lost foam and

sand core casting method that includes the step of forming a core of bonded granular material, preferably sand or ceramic, containing voids. The core has voids formed in it that have at least two exposed sides. A first layer of lost foam destructible material is then preformed in a separate mold, preferably by an injection process. Similarly, a second layer of lost foam destructible material is preformed.

The first foam layer is positioned on one side of the core, and the second foam layer is positioned on another side of the core. The layers are glued to the core, closing off the exposed sides of the voids formed in the core.

The assembly is attached to a down sprue and lowered in a mold cavity, which is then packed with a mold media that is preferably the same as the media of the core. The assembly is vibration compacted and/or vacuum compacted within the ceramic and/or sand media. The foam layers prevent entry of mold media into the voids. Molten metal is then delivered to the mold cavity to form the casting. The lost foam layers are gasified and replaced by the molten metal as it enters the mold. The voids in the core as well as the spaces previously occupied by the foam layers are filled with the advancing molten metal. After cooling, the cast component is removed from the mold cavity, and the material of the core, which is no longer bonded, is removed from the component.

### BRIEF DESCRIPTION OF THE DRAWINGS

FIG. 1 is a cross-sectional, exploded and simplified elevation view of a core, an upper lost foam mold, and a lower lost foam layer constructed in accordance with this invention.

FIG. 2 is a cross-sectional and simplified elevation view of an assembly comprised of the core, upper lost foam layer, and lower lost foam layer of FIG. 1.

FIG. 3 is a side view of a plurality of the assemblies of FIG. 2 lowered into a molding flask on a down sprue.

FIG. 4 is a top view of the core shown in FIGS. 1 and 2.

FIG. 5 is a bottom view of the core shown in FIGS. 1 and 2.

FIG. 6 is a cross-sectional view of a finished pump impeller formed from the assembly of FIG. 2.

FIG. 7 is a cross-sectional view of a finished diffuser formed from a method in accordance with this invention.

### DETAILED DESCRIPTION OF THE INVENTION

Referring now to FIGS. 1 and 2, core **10** is formed of a bonded granular material, preferably chemically bonded mullite. Mullite is a type of fine grade ceramic material. However, sand or other materials may be used, including silica sand and a binder such as phenolic base and/or modified phenolic base resin. Core **10** may be formed by a variety of conventional techniques. The material of the first core **10** should be compacted sufficiently to act as a backing that will generate enough mold strength in conjunction with the mullite media to create a hydraulically sound part with a near net shape configuration.

Core **10** is shaped for forming cavities in a centrifugal pump impeller, and is shown in a simplified manner in FIG. 1, rather than with curved contours that would exist in practice. Core **10** is in a circular disk-shaped configuration with a central axis, an upward extending central cylindrical hub portion **11** and a radially extending flange **12**. The terms "upper" or "upward" and "lower" or "downward" are used for convenience herein and not in a limiting manner. A depending lip **13** extends around the circumference of flange

12. A solid downward extending mandrel **14** extends from the lower side of core **10**. An annular recess **15** with a closed upper surface is formed in the lower side of core **10**, encircling mandrel **14**.

Flange **12** is formed with a plurality of voids or spaces **16** as shown in FIG. 4. Voids **16** extend from upper hub **11** outward in a spiral or helical pattern. Each void **16** extends completely through flange **12**, and has an outer end that is closed by lip **13**, which extends in a continuous uninterrupted circle around flange **12**. Consequently, voids **16** have exposed upper and lower sides. Voids **16** are fairly thin in width and define fingers **17** in core **10** between them that are wider considerably than voids **16**.

A protective core wash may be used to coat the surface of core **10** to enhance the surface finish of the casting. The particular core wash is customized for use with a particular alloy to minimize interaction and to meet specific permeability requirements as is known in the art.

An upper lost foam layer **18** is preformed of a cellular plastic foam material of a type that will vaporize when contacted by hot metal. The destructible material of upper lost foam layer **18** may be any type of suitable low temperature fusible substance, including a thermoplastic resinous material or any other cellular plastic material that gasifies substantially without residue. Materials that may be used include polystyrene and resinous polymerized derivatives of methacrylic acid. Various types of cellular plastic materials suitable for use in casting operations are taught in the following U.S. patents: U.S. Pat. No. 3,374,827, issued to Schlebler on Mar. 26, 1968, and U.S. Pat. No. 3,496,989, issued to Paoli on Feb. 24, 1970. The expression "destructible" as applied to the cellular plastic layer is intended to refer to materials that are quickly destroyed by molten metal. The destructible nature of the materials enables the molten metal to occupy the space originally occupied by the destructible material. In contrast, the "core" material is "non-destructible" in the sense that the core material is able to resist the effects of the molten metal. Therefore, the core material produces a cavity in the casting.

Upper lost foam layer **18** has a radially extending flat flange **24** and a central upward extending hub **20**. Unlike flange **12** of core **10**, there are no voids in flange **24**, rather it is solid and has flat, smooth upper and lower surfaces. An opening **22** extends through hub **20** and is sized for close reception over upper hub portion **11** of core **10**. The height of hub **20** of upper lost foam layer **18** is less than the height of upper hub **11** in the embodiment shown.

A lower lost foam layer **26** of the same material as upper lost foam layer **18** is also preformed. Lower lost foam layer **26** has a central hub **28** with a passage **29** extending through it. A flat circular flange **30** extends radially outward from hub **28** at a point between the upper and lower ends of hub **28**. Flange **30** is also solid with substantially flat upper and lower surfaces. Hub **28** is sized to fit closely in recess **15**. Mandrel **14** of core **10** fits closely within passage **29** and protrudes slightly below the lower end of hub **28**.

Upper and lower foam layers **18, 26** may be preformed a variety of manners. Preferably, they are formed by injection molding techniques in an aluminum mold. Beads of cellular plastic material are injected into cavities in the aluminum mold, then expanded by the application of steam.

In practice, the preformed upper lost foam layer **18** is affixed to the upper side of the core **10**, preferably by an adhesive, as shown in FIG. 2. The preformed lower lost foam layer **26** is positioned and affixed to the lower side of core **10** by adhesive, as shown in FIG. 2. The periphery of

flange **30** locates within lip **13**, and hub **28** extends into core recess **15**. Once assembled as in FIG. 2, flange **24** of upper foam layer **18** will close the upper sides of voids **16** (FIGS. 4, 5), and flange **30** of lower foam layer **26** will close the lower sides of voids **16**. Core lip **13** encloses the outer ends of voids **16**. Voids **16** are thus completely sealed.

The assembly **31** of core **10**, and foam layers **18** and **26** are attached to a down sprue **34** (FIG. 3) and lowered into a flask **36**. FIG. 3 shows eight of the assemblies **31** mounted to down sprue **34** and being simultaneously positioned in flask **36**. A refractory molding media **38** is packed around assemblies **31**. Molding media **38** is preferably the same as the material of core **10**, such as ceramic mullite. The molding media **38** is unbonded and either vacuum and/or vibration compacted in place. The media **38** closely contacts and forms to the configuration of the assemblies **31**.

Molten metal is then delivered to the assemblies **31** through a sprue cup **40** and down sprues **34** to form a casting of a workpiece or component, such as an impeller or diffuser.

The upper lost foam layer **18** and lower lost foam layer **26** are gasified and replaced by the molten metal as it enters the mold. Voids **16** in core **10** (FIGS. 4 and 5) are also filled with the advancing molten metal. After cooling, the component is removed, and the granular media of core **10** is shaken from or otherwise removed from the component. This leaves a plurality of passages in the component where fingers **17** (FIGS. 4, 5) previously existed. Voids **16** resulted in lateral sidewalls being formed for the passages of the component, while foam layers **18, 26** resulted in upper and lower walls of the passages of the component.

An assembly similar to assembly **31**, but more contoured, will form an impeller **42**, shown in FIG. 6. Impeller **42** has helical passages **44** formed therein by fingers **17** (FIGS. 4, 5) of core **10** and upper and lower layers **18, 26**. Impeller **42** has a hub **46** formed by corresponding portions of assembly **31**.

An assembly (not shown) formed in the same manner, with a core of bonded granular material and upper and lower lost foam layers will also form a diffuser **48**, shown in FIG. 7. Diffuser **48** has a central portion **50** and a plurality of passages **52** formed therein. Impeller **42** and diffuser **48** form a pump stage of a centrifugal pump.

The method of the invention has several advantages. By preforming the destructible material layers, then gluing the destructible material layers to a core, moisture from the steam expansion step never contacts the bonded granular material core. Additionally, the interior of the resulting casting is smooth-surfaced, free of pits and fins.

An important advantage is the use of voids in the core that are initially sealed by the foam layers, then filled with metal as the metal is introduced into the mold. The method of the invention requires no gluing lines that might occur when gluing two sand cores together. The absence of gluing lines results in an improved surface finish and dimensional stability. A casting with a complex internal geometry having a high level of surface finish may be formed. The result is a casting of complex internal geometry with a very high level of surface finish as cast, which yields improved hydraulic performance.

While the invention has been shown in only one of its forms, it should be apparent to those skilled in the art that it is not so limited, but is susceptible to various changes without departing from the scope of the invention.

What is claimed is:

1. A method of casting a workpiece having at least one cavity, comprising:

- (a) performing a core of bonded granular material in the desired configuration of the cavity of the workpiece, the core having at least one core cavity formed therein which has at least one exposed side;
  - (b) performing a fusible member, then positioning the fusible member over the exposed side of said core cavity, forming an assembly;
  - (c) placing the assembly in a refractory mold cavity and packing granular refractory medial around the assembly, with the fusible member blocking entry of the refractory media into said core cavity, leaving said core cavity unfilled;
  - (d) delivering molten metal into the mold cavity into contact with the fusible member, which decomposes, causing the molten metal to flow into said core cavity, forming a metal wall of the workpiece in said core cavity and in the space previously occupied by the fusible member; then
  - (e) removing the workpiece and the core from the mold cavity and removing the bonded granular material of the core from the workpiece.
2. The method according to claim 1, wherein the fusible member is secured adhesively to the core in step (b).
3. The method according to claim 1, wherein:
- step (a) further comprises forming a recess in the core; and step (b) further comprises performing a protrusion on the fusible member of a shape that matches the recess and inserting the protrusion into the recess.
4. The method according to claim 1, wherein:
- step (a) further comprises performing a mandrel on the core; and
  - step (b) further comprises performing a hole in the fusible member and inserting the mandrel into the hole.
5. A method of casting a workpiece having at least one cavity therein, comprising:
- (a) performing a core of bonded granular material in the desired configuration of the cavity of the workpiece, the core having oppositely facing first and second surfaces with at least one core cavity extending between the first and second surfaces, said core cavity having exposed sides at the first and second surfaces and being in the desired configuration of a wall for the workpiece;
  - (b) performing a first foam fusible member of fusible material, then positioning the first foam fusible member on the first surface of the core, overlying and closing off one of the exposed sides of said core cavity;
  - (c) performing a second foam fusible member of fusible material, then positioning the second foam fusible member on the second surface of the core, overlying and closing off an opposite one of the exposed sides of said core cavity, forming an assembly of the first and second foam molds with the core, leaving said core cavity unfilled;
  - (d) placing the assembly in a refractory mold cavity and packing granular refractory material around the assembly;
  - (e) delivering molten metal into the mold cavity into contact with the first and second foam fusible members, which decompose, causing the molten metal to flow into said core cavity, forming a metal wall for the workpiece in said core cavity and in the spaces previously occupied by the foam fusible members; then
  - (f) removing the workpiece and the core from the mold cavity and removing the bonded granular material of

- the core from the workpiece, providing the desired cavity for the workpiece.
6. The method according to claim 5, wherein in step (c), the foam fusible members are adhesively secured to the core.
7. The method according to claim 5, wherein in step (d) the molten metal flowing into said core cavity forms a side wall of the cavity of the workpiece, and the molten metal flowing into the spaces occupied by the first and second fusible members forms upper and lower walls of the cavity of the workpiece, the upper and lower walls being joined to each other by the side wall.
8. The method according to claim 5, wherein:
- step (a) further comprises forming a recess in the second surface;
  - and step (c) further comprises performing a protrusion on the second foam fusible member of a shape that matches the recess and inserting the protrusion into the recess.
9. The method according to claim 5, wherein:
- step (a) further comprises performing a mandrel on the second surface of the core; and
  - step (c) further comprises performing a hole in the second foam fusible member and inserting the mandrel into the hole.
10. A method of casting a centrifugal pump stage component having a plurality of a plurality of passages extending outward from a central axis, each of the passages being defined by sidewalls and first and second oppositely facing walls, the method comprising:
- (a) forming a core of bonded granular material, having outward extending fingers separated by core cavities, each of the fingers being in the configuration of one of the passages of the component, and each of said core cavities being in the configuration of one of the sidewalls of the component, said core cavities having first and second exposed sides;
  - (b) performing a first foam fusible member of fusible material, then positioning the first foam fusible member on a first surface of the core in contact with the fingers, overlying and closing off the first exposed sides of said core cavities, the first foam fusible member having portions in the configuration of the first walls of the passages of the component;
  - (c) performing a second foam fusible member of fusible material, then positioning the second foam fusible member on a second surface of the core in contact with the fingers, overlying and closing off the second exposed sides of said core cavities, the second foam fusible member having portions in the configuration of the second walls of the passages of the component, the foam fusible members and the core forming an assembly, leaving said core cavities unfilled;
  - (d) placing the assembly in a refractory mold cavity and packing granular refractory material around the assembly;
  - (e) delivering molten metal into the mold cavity into contact with the first and second foam fusible members, which decompose, causing the molten metal to flow into said core cavities, forming sidewalls for the passages of the component in said core cavities and forming first and second walls for the passages in the spaces previously occupied by the foam fusible members; then
  - (f) removing the component and the core from the mold cavity and removing the bonded granular material of

the core from the component, providing the desired passages for the component.

11. The method according to claim 10, wherein in step (c), the foam fusible members are adhesively secured to the core.

12. The method according to claim 10, wherein in step (d) the molten metal flowing into said core cavities and spaces joins the sidewalls of the passages with the first and second walls of the passages.

13. The method according to claim 10, wherein:

step (a) further comprises forming a recess in the core; and step (c) further comprises preforming a protrusion on the second foam fusible member of a shape that matches the recess and inserting the protrusion into the recess.

14. The method according to claim 10, wherein: step (a) further comprises preforming a mandrel on the core; and

step (c) further comprises preforming a hole in the second foam fusible member and inserting the mandrel into the hole.

15. The method according to claim 10, wherein in step (a), the fingers of the core are formed to extend outward in a spiral pattern.

16. The method according to claim 10, wherein in step (a), the fingers and the openings of the core are formed to extend outward in a spiral pattern, and wherein the core is formed with an annular lip surrounding outward ends of said core cavities and joining outward ends of the fingers.

\* \* \* \* \*

UNITED STATES PATENT AND TRADEMARK OFFICE  
**CERTIFICATE OF CORRECTION**

PATENT NO. : 6,305,458 B1  
DATED : October 23, 2001  
INVENTOR(S) : Corneliu Ioan Gligor

Page 1 of 1

It is certified that error appears in the above-identified patent and that said Letters Patent is hereby corrected as shown below:

Column 5.  
Line 9, delete "medial" and insert -- media --.

Signed and Sealed this

Twenty-eighth Day of May, 2002

*Attest:*



*Attesting Officer*

JAMES E. ROGAN  
*Director of the United States Patent and Trademark Office*